



US010760151B2

(12) **United States Patent**  
**Doud et al.**

(10) **Patent No.:** **US 10,760,151 B2**  
(45) **Date of Patent:** **\*Sep. 1, 2020**

(54) **GALVANICALLY-ACTIVE IN SITU FORMED PARTICLES FOR CONTROLLED RATE DISSOLVING TOOLS**

(71) Applicant: **Terves Inc.**, Euclid, OH (US)

(72) Inventors: **Brian P. Doud**, Cleveland Heights, OH (US); **Nicholas J. Farkas**, Euclid, OH (US); **Andrew J. Sherman**, Mentor, OH (US)

(73) Assignee: **Terves, LLC**, Euclid, OH (US)

(\*) Notice: Subject to any disclaimer, the term of this patent is extended or adjusted under 35 U.S.C. 154(b) by 153 days.

This patent is subject to a terminal disclaimer.

(21) Appl. No.: **15/888,751**

(22) Filed: **Feb. 5, 2018**

(65) **Prior Publication Data**

US 2018/0155813 A1 Jun. 7, 2018

**Related U.S. Application Data**

(62) Division of application No. 14/689,295, filed on Apr. 17, 2015, now Pat. No. 9,903,010.  
(Continued)

(51) **Int. Cl.**  
**C22F 1/06** (2006.01)  
**C22C 1/02** (2006.01)  
(Continued)

(52) **U.S. Cl.**  
CPC ..... **C22F 1/06** (2013.01); **C22C 1/02** (2013.01); **C22C 23/02** (2013.01); **C22C 23/00** (2013.01)

(58) **Field of Classification Search**  
CPC ... C22F 1/06; C22C 23/02; C22C 1/02; C22C 23/00

See application file for complete search history.

(56) **References Cited**

**U.S. PATENT DOCUMENTS**

3,180,728 A 4/1965 Pryor et al.  
3,445,731 A 5/1969 Saeki et al.  
(Continued)

**FOREIGN PATENT DOCUMENTS**

CA 2886988 10/2015  
CN 101381829 3/2009  
(Continued)

**OTHER PUBLICATIONS**

Sigworth et al. "Grain Refinement of Aluminum Castings Alloys" American Foundry Society; Paper 07-67; pp. 5-7 (2007).

(Continued)

*Primary Examiner* — Anthony J Zimmer

(74) *Attorney, Agent, or Firm* — Fay Sharpe LLP

**ABSTRACT**

A castable, moldable, and/or extrudable structure using a metallic primary alloy. One or more additives are added to the metallic primary alloy so that in situ galvanically-active reinforcement particles are formed in the melt or on cooling from the melt. The composite contain an optimal composition and morphology to achieve a specific galvanic corrosion rate in the entire composite. The in situ formed galvanically-active particles can be used to enhance mechanical properties of the composite, such as ductility and/or tensile strength. The final casting can also be enhanced by heat treatment, as well as deformation processing such as extrusion, forging, or rolling, to further improve the strength of the final composite over the as-cast material.

**100 Claims, 4 Drawing Sheets**



| Related U.S. Application Data |                                                                 |              |    |         |                 |  |
|-------------------------------|-----------------------------------------------------------------|--------------|----|---------|-----------------|--|
| (60)                          | Provisional application No. 61/981,425, filed on Apr. 18, 2014. | 9,187,686    | B2 | 11/2015 | Crews           |  |
|                               |                                                                 | 9,217,319    | B2 | 12/2015 | Frazier et al.  |  |
|                               |                                                                 | 9,227,243    | B2 | 1/2016  | Xu et al.       |  |
|                               |                                                                 | 9,243,475    | B2 | 1/2016  | Xu              |  |
|                               |                                                                 | 9,309,744    | B2 | 4/2016  | Frazier         |  |
|                               |                                                                 | 9,447,482    | B2 | 9/2016  | Kim et al.      |  |
| (51)                          | <b>Int. Cl.</b>                                                 | 9,528,343    | B2 | 12/2016 | Jordan et al.   |  |
|                               | <i>C22C 23/02</i> (2006.01)                                     | 9,605,508    | B2 | 3/2017  | Xu              |  |
|                               | <i>C22C 23/00</i> (2006.01)                                     | 9,938,451    | B2 | 4/2018  | Crews           |  |
| (56)                          | <b>References Cited</b>                                         | 2002/0102179 | A1 | 8/2002  | Murai           |  |
|                               | U.S. PATENT DOCUMENTS                                           | 2002/0121081 | A1 | 9/2002  | Cesaroni et al. |  |
|                               |                                                                 | 2002/0197181 | A1 | 12/2002 | Osawa et al.    |  |
|                               |                                                                 | 2003/0173005 | A1 | 9/2003  | Higashi         |  |
|                               |                                                                 | 2005/0194141 | A1 | 9/2005  | Sinclair et al. |  |
|                               |                                                                 | 2006/0113077 | A1 | 6/2006  | Willberg et al. |  |
|                               |                                                                 | 2006/0131031 | A1 | 6/2006  | McKeachnie      |  |
|                               |                                                                 | 2006/0175059 | A1 | 8/2006  | Sinclair et al. |  |
|                               |                                                                 | 2006/0207387 | A1 | 9/2006  | Soran et al.    |  |
|                               |                                                                 | 2006/0278405 | A1 | 12/2006 | Turley          |  |
|                               |                                                                 | 2007/0181224 | A1 | 8/2007  | Marya et al.    |  |
|                               |                                                                 | 2008/0041500 | A1 | 2/2008  | Bronfin         |  |
|                               |                                                                 | 2008/0149345 | A1 | 6/2008  | Marya et al.    |  |
|                               |                                                                 | 2008/0175744 | A1 | 7/2008  | Motegi          |  |
|                               |                                                                 | 2009/0116992 | A1 | 5/2009  | Lee             |  |
|                               |                                                                 | 2009/0226340 | A1 | 9/2009  | Marya           |  |
|                               |                                                                 | 2010/0119405 | A1 | 5/2010  | Okamoto et al.  |  |
|                               |                                                                 | 2010/0161031 | A1 | 6/2010  | Papirov et al.  |  |
|                               |                                                                 | 2010/0270031 | A1 | 10/2010 | Patel           |  |
|                               |                                                                 | 2010/0304178 | A1 | 12/2010 | Dirscherl       |  |
|                               |                                                                 | 2011/0048743 | A1 | 3/2011  | Stafford et al. |  |
|                               |                                                                 | 2011/0067889 | A1 | 3/2011  | Marya et al.    |  |
|                               |                                                                 | 2011/0091660 | A1 | 4/2011  | Dirscherl       |  |
|                               |                                                                 | 2011/0135530 | A1 | 6/2011  | Xu et al.       |  |
|                               |                                                                 | 2011/0221137 | A1 | 9/2011  | Obi et al.      |  |
|                               |                                                                 | 2011/0236249 | A1 | 9/2011  | Kim et al.      |  |
|                               |                                                                 | 2012/0080189 | A1 | 4/2012  | Marya et al.    |  |
|                               |                                                                 | 2012/0097384 | A1 | 4/2012  | Valencia et al. |  |
|                               |                                                                 | 2012/0103135 | A1 | 5/2012  | Xu et al.       |  |
|                               |                                                                 | 2012/0125642 | A1 | 5/2012  | Chenault        |  |
|                               |                                                                 | 2012/0156087 | A1 | 6/2012  | Kawabata        |  |
|                               |                                                                 | 2012/0177905 | A1 | 7/2012  | Seals et al.    |  |
|                               |                                                                 | 2012/0190593 | A1 | 7/2012  | Soane et al.    |  |
|                               |                                                                 | 2012/0273229 | A1 | 11/2012 | Xu et al.       |  |
|                               |                                                                 | 2012/0318513 | A1 | 12/2012 | Mazyar et al.   |  |
|                               |                                                                 | 2013/0022816 | A1 | 1/2013  | Smith et al.    |  |
|                               |                                                                 | 2013/0029886 | A1 | 1/2013  | Mazyar et al.   |  |
|                               |                                                                 | 2013/0032357 | A1 | 2/2013  | Mazyar et al.   |  |
|                               |                                                                 | 2013/0043041 | A1 | 2/2013  | McCoy et al.    |  |
|                               |                                                                 | 2013/0047785 | A1 | 2/2013  | Xu              |  |
|                               |                                                                 | 2013/0056215 | A1 | 3/2013  | Crews           |  |
|                               |                                                                 | 2013/0068411 | A1 | 3/2013  | Forde et al.    |  |
|                               |                                                                 | 2013/0112429 | A1 | 5/2013  | Crews           |  |
|                               |                                                                 | 2013/0133897 | A1 | 5/2013  | Bailhly et al.  |  |
|                               |                                                                 | 2013/0160992 | A1 | 6/2013  | Agrawal et al.  |  |
|                               |                                                                 | 2013/0168257 | A1 | 7/2013  | Mazyar et al.   |  |
|                               |                                                                 | 2013/0199800 | A1 | 8/2013  | Kellner et al.  |  |
|                               |                                                                 | 2013/0209308 | A1 | 8/2013  | Mazyar et al.   |  |
|                               |                                                                 | 2013/0220496 | A1 | 8/2013  | Inoue           |  |
|                               |                                                                 | 2013/0261735 | A1 | 10/2013 | Pacetti et al.  |  |
|                               |                                                                 | 2013/0048289 | A1 | 12/2013 | Mazyar          |  |
|                               |                                                                 | 2014/0018489 | A1 | 1/2014  | Johnson         |  |
|                               |                                                                 | 2014/0027128 | A1 | 1/2014  | Johnson         |  |
|                               |                                                                 | 2014/0060834 | A1 | 3/2014  | Quintero        |  |
|                               |                                                                 | 2014/0093417 | A1 | 4/2014  | Liu             |  |
|                               |                                                                 | 2014/0124216 | A1 | 5/2014  | Fripp et al.    |  |
|                               |                                                                 | 2014/0190705 | A1 | 7/2014  | Fripp           |  |
|                               |                                                                 | 2014/0196889 | A1 | 7/2014  | Jordan et al.   |  |
|                               |                                                                 | 2014/0202284 | A1 | 7/2014  | Kim             |  |
|                               |                                                                 | 2014/0202708 | A1 | 7/2014  | Jacob et al.    |  |
|                               |                                                                 | 2014/0219861 | A1 | 8/2014  | Han             |  |
|                               |                                                                 | 2014/0224477 | A1 | 8/2014  | Wiese et al.    |  |
|                               |                                                                 | 2014/0236284 | A1 | 8/2014  | Stinson         |  |
|                               |                                                                 | 2014/0271333 | A1 | 9/2014  | Kim et al.      |  |
|                               |                                                                 | 2014/0286810 | A1 | 9/2014  | Marya           |  |
|                               |                                                                 | 2014/0305627 | A1 | 10/2014 | Manke           |  |
|                               |                                                                 | 2015/0102179 | A1 | 4/2015  | McHenry et al.  |  |
|                               |                                                                 | 2015/0240337 | A1 | 8/2015  | Sherman et al.  |  |
|                               |                                                                 | 2015/0247376 | A1 | 9/2015  | Tolman          |  |

(56)

## References Cited

## U.S. PATENT DOCUMENTS

|                  |         |               |           |
|------------------|---------|---------------|-----------|
| 2015/0299838 A1* | 10/2015 | Doud .....    | C22F 1/06 |
|                  |         |               | 420/409   |
| 2015/0354311 A1  | 12/2015 | Okura et al.  |           |
| 2016/0024619 A1  | 1/2016  | Wilks         |           |
| 2016/0201425 A1  | 7/2016  | Walton        |           |
| 2016/0201427 A1  | 7/2016  | Fripp         |           |
| 2016/0201435 A1  | 7/2016  | Fripp et al.  |           |
| 2016/0230494 A1  | 8/2016  | Fripp         |           |
| 2016/0251934 A1  | 9/2016  | Walton et al. |           |
| 2016/0265091 A1  | 9/2016  | Walton et al. |           |

## FOREIGN PATENT DOCUMENTS

|    |              |         |
|----|--------------|---------|
| CN | 102517489    | 6/2012  |
| CN | 102796928    | 11/2012 |
| CN | 103343271    | 10/2013 |
| CN | 103602865    | 2/2014  |
| CN | 103898384    | 7/2014  |
| EP | 0470599      | 2/1998  |
| EP | 2088217      | 8/2009  |
| JP | 2008266734   | 11/2008 |
| JP | 2012197491   | 10/2012 |
| JP | 2013019030   | 1/2013  |
| JP | 2014043601   | 3/2014  |
| KR | 20130023707  | 3/2013  |
| WO | US1990002655 | 3/1990  |
| WO | 1992013978   | 8/1992  |
| WO | 9857347      | 12/1998 |
| WO | 1999027146   | 6/1999  |
| WO | 2009055354   | 4/2009  |
| WO | 2009093420   | 7/2009  |
| WO | 2012091984   | 7/2012  |
| WO | 2013019410   | 2/2013  |
| WO | 2013019421   | 2/2013  |
| WO | 2013109287   | 7/2013  |
| WO | 2013122712   | 8/2013  |
| WO | 2013154634   | 10/2013 |
| WO | 2014100141   | 6/2014  |
| WO | 2014113058   | 7/2014  |
| WO | 2015171126   | 11/2015 |
| WO | 2016032758   | 3/2016  |
| WO | 2016032761   | 3/2016  |
| WO | 2016036371   | 3/2016  |

## OTHER PUBLICATIONS

- Momentive, "Titanium Diborid Powder" condensed product brochure; retrieved from <https://www.momentive.com/WorkArea/DownloadAsset.aspx?id=27489>; p. 1 (2012).
- Durbin, "Modeling Dissolution in Aluminum Alloys" Dissertation for Georgia Institute of Technology; retrieved from [https://smartech.gatech.edu/bitstream/handle/1853/6873/durbin\\_tracie\\_L\\_200505\\_phd.pdf](https://smartech.gatech.edu/bitstream/handle/1853/6873/durbin_tracie_L_200505_phd.pdf) (2005).
- Pegeut et al., "Influence of cold working on the pitting corrosion resistance of stainless steel" Corrosion Science, vol. 49, pp. 1933-1948 (2007).
- Elemental Charts from [chemicalelements.com](http://chemicalelements.com); retrieved Jul. 27, 2017.
- Song et al., "Corrosion Mechanisms of Magnesium Alloys" Advanced Engg Materials, vol. 1, No. 1 (1999).
- Zhou et al., "Tensile Mechanical Properties and Strengthening Mechanism of Hybrid Carbon Nanotubes . . ." Journal of Nanomaterials, 2012; 2012:851862 (doi: 10.1155/2012/851862) Figs. 6 and 7.
- Trojanova et al., "Mechanical and Acoustic Properties of Magnesium Alloys . . ." Light Metal Alloys Application, Chapter 8, Published Jun. 11, 2014 (doi: 10.5772/57454) p. 163, para. [0008], [0014-0015]; [0041-0043].
- AZoNano "Silicon Carbide Nanoparticles—Properties, Applications" <http://www.amazon.com/articles.aspx?ArticleID=3396> p. 2, Physical Properties, Thermal Properties (May 9, 2013).
- AZoM "Magnesium AZ91D-F Alloy" <http://www.amazon.com/articles.aspx?ArticleID=8670> p. 1, Chemical Composition; p. 2 Physical Properties (Jul. 31, 2013).
- Elasser et al., "Silicon Carbide Benefits and Advantages . . ." Proceedings of the IEEE, 2002; 906(6):969-986 (doi: 10.1109/JPROC2002.1021562) p. 970, Table 1.
- Lan et al., "Microstructure and Microhardness of SiC Nanoparticles . . ." Materials Science and Engineering A; 386:284-290 (2004).
- Casati et al., "Metal Matrix Composites Reinforced by Nanoparticles", vol. 4:65-83 (2014).
- Saravanan et al., "Fabrication and characterization of pure magnesium-30 vol. SiCP particle composite", Material Science and Eng., vol. 276, pp. 108-116 (2000).
- Song et al., Texture evolution and mechanical properties of AZ31B magnesium alloy sheets processed by repeated unidirectional bending, Journal of Alloys and Compounds, vol. 489, pp. 475-481 (2010).
- Blawert et al., "Magnesium secondary alloys: Alloy design for magnesium alloys with improved tolerance limits against impurities", Corrosion Science, vol. 52, No. 7, pp. 2452-2468 (Jul. 1, 2010).
- Wang et al., "Effect of Ni on microstructures and mechanical properties of AZ1 02 magnesium alloys" Zhuzao Foundry, Shenyang Zhuzao Yanjusuo, vol. 62, No. 1, pp. 315-318 (Jan. 1, 2013).
- Kim et al., "Effect of aluminum on the corrosion characteristics of Mg—4Ni—xAl alloys", Corrosion, vol. 59, No. 3, pp. 228-237 (Jan. 1, 2003).
- Unsworth et al., "A new magnesium alloy system", Light Metal Age, vol. 37, No. 7-8., pp. 29-32 (Jan. 1, 1979).
- Geng et al., "Enhanced age-hardening response of Mg—Zn alloys via Co additions", Scripta Materialia, vol. 64, No. 6, pp. 506-509 (Mar. 1, 2011).
- Zhu et al., "Microstructure and mechanical properties of Mg6ZnCuO.6Zr (wt.%) alloys", Journal of Alloys and Compounds, vol. 509, No. 8, pp. 3526-3531 (Dec. 22, 2010).
- International Search Authority, International Search Report and Written Opinion for PCT/GB2015/052169 (dated Feb. 17, 2016). Search and Examination Report for GB 1413327.6 (dated Jan. 21, 2015).
- Magnesium Elektron Test Report (dated Mar. 8, 2005).
- New England Fishery Management Counsel, "Fishery Management Plan for American Lobster Amendment 3" (Jul. 1989).
- Emly, E.F., "Principles of Magnesium Technology" Pergamon Press, Oxford (1966).
- Shaw, "Corrosion Resistance of Magnesium Alloys", ASM Handbook, vol. 13A, pp. 692-696 (2003).
- Hanawalt et al., "Corrosion studies of magnesium and its alloys", Metals Technology, Technical Paper 1353 (1941).
- The American Foundry Society, Magnesium alloys, casting source directory 8208, available at [www.afsinc.org/files/magnes.pdf](http://www.afsinc.org/files/magnes.pdf).
- Rokhlin, "Magnesium alloys containing rare earth metals structure and properties", Advances in Metallic Alloys, vol. 3, Taylor & Francis (2003).
- Ghali, "Corrosion Resistance of Aluminum and Magnesium Alloys" pp. 382-389, Wiley Publishing (2010).
- Kim et al., "High Mechanical Strengths of Mg—Ni—Y and MG—Cu Amorphous Alloys with Significant Supercooled Liquid Region", Materials Transactions, vol. 31, No. 11, pp. 929-934 (1990).
- Tekumalla et al., "Mechanical Properties of Magnesium—Rare Earth Alloy Systems", Metals, vol. 5, pp. 1-39 (2014).
- National Physical Laboratory, "Bimetallic Corrosion" Crown (C) p. 1-14 (2000).
- Ye et al., "Review of recent studies in magnesium matrix composites", Journal of Material Science, vol. 39, pp. 6153-6171 (2004).
- Hassan et al., "Development of a novel magnesium-copper based composite with improved mechanical properties", Materials Research Bulletin, vol. 37, pp. 377-389 (2002).
- Ye et al., "Microstructure and tensile properties of Ti6Al4V/AM60B magnesium matrix composite", Journal of Alloys and Composites, vol. 402, pp. 162-169 (2005).
- Kumar et al., "Mechanical and Tribological Behavior of Particulate Reinforced Aluminum metal Matrix Composite", Journal of Minerals & Materials Characterization and Engineering, vol. 10, pp. 59-91 (2011).

(56)

**References Cited**

OTHER PUBLICATIONS

- Majumdar, "Micromechanics of Discontinuously Reinforced MMCs", Engineering Mechanics and Analysis of Metal-Matrix Composites, vol. 21, pp. 395-406.
- Scharf et al., "Corrosion of AX 91 Secondary Magnesium Alloy", Advanced Engineering Materials, vol. 7, No. 12, pp. 1134-1142 (2005).
- Hillis et al., "High Purity Magnesium AM60 Alloy: The Critical Contaminant Limits and the Salt Water Corrosion Performance", SAE Technical Paper Series (1986).
- Pawar, S.G., "Influence of Microstructure on the Corrosion Behaviour of Magnesium Alloys", PhD Dissertation, University of Manchester (2011).
- Czerwinski, "Magnesium Injection Molding"; Technology & Engineering; Springer Science + Media, LLC, pp. 107-108, (Dec. 2007).
- Metals Handbook, Desk Edition, edited by J.R. Davis, published by ASM International, pp. 559-574 (1998).

\* cited by examiner



FIG 1.



FIG. 2



Highlighted In Situ Formed Particles

**FIG. 3**



FIG. 4

**GALVANICALLY-ACTIVE IN SITU FORMED  
PARTICLES FOR CONTROLLED RATE  
DISSOLVING TOOLS**

The present invention is a divisional of U.S. patent application Ser. No. 14/689,295 filed Apr. 17, 2015, which in turn claims priority on U.S. Provisional Patent Application Ser. No. 61/981,425 filed Apr. 18, 2014, which is incorporated herein by reference.

**FIELD OF THE INVENTION**

The present invention is directed to a novel magnesium composite for use as a dissolvable component in oil drilling.

**BACKGROUND OF THE INVENTION**

The ability to control the dissolution of a down hole well component in a variety of solutions is very important to the utilization of non-drillable completion tools, such as sleeves, frac balls, hydraulic actuating tooling, and the like. Reactive materials for this application, which dissolve or corrode when exposed to acid, salt, and/or other wellbore conditions, have been proposed for some time. Generally, these components consist of materials that are engineered to dissolve or corrode. Dissolving polymers and some powder metallurgy metals have been disclosed, and are also used extensively in the pharmaceutical industry for controlled release of drugs. Also, some medical devices have been formed of metals or polymers that dissolve in the body.

While the prior art well drill components have enjoyed modest success in reducing well completion costs, their consistency and ability to specifically control dissolution rates in specific solutions, as well as other drawbacks such as limited strength and poor reliability, have impacted their ubiquitous adoption. Ideally, these components would be manufactured by a process that is low cost, scalable, and produces a controlled corrosion rate having similar or increased strength as compared to traditional engineering alloys such as aluminum, magnesium, and iron. Ideally, traditional heat treatments, deformation processing, and machining techniques could be used on the components without impacting the dissolution rate and reliability of such components.

**SUMMARY OF THE INVENTION**

The present invention is directed to a novel magnesium composite for use as a dissolvable component in oil drilling and will be described with particular reference to such application. As can be appreciated, the novel magnesium composite of the present invention can be used in other applications (e.g., non-oil wells, etc.). In one non-limiting embodiment, the present invention is directed to a ball or other tool component in a well drilling or completion operation such as, but not limited to, a component that is seated in a hydraulic operation that can be dissolved away after use so that no drilling or removal of the component is necessary. Tubes, valves, valve components, plugs, frac balls, and other shapes and components can "also be formed of the novel magnesium composite of the present invention. For purposes of this invention, primary dissolution is measured for valve components and plugs as the time the part removes itself from the seat of a valve or plug arrangement or can become free floating in the system. For example, when the part is a plug in a plug system, primary dissolution occurs when the plug has degraded or dissolved to a point

that it can no longer function as a plug and thereby allows fluid to flow about the plug. For purposes of this invention, secondary dissolution is measured in the time the part is fully dissolved into sub-mm particles. As can be appreciated, the novel magnesium composite of the present invention can be used in other well components that also desire the function of dissolving after a period of time. In one non-limiting aspect of the present invention, a galvanically-active phase is precipitated from the novel magnesium composite composition and is used to control the dissolution rate of the component; however, this is not required. The novel magnesium composite is generally castable and/or machinable, and can be used in place of existing metallic or plastic components in oil and gas drilling rigs including, but not limited to, water injection and hydraulic fracturing. The novel magnesium composite can be heat treated as well as extruded and/or forged.

In one non-limiting aspect of the present invention, the novel magnesium composite is used to form a castable, moldable, or extrudable component. Non-limiting magnesium composites in accordance with the present invention include at least 50 wt. % magnesium. One or more additives are added to a magnesium or magnesium alloy to form the novel magnesium composite of the present invention. The one or more additives can be selected and used in quantities so that galvanically-active intermetallic or insoluble precipitates form in the magnesium or magnesium alloy while the magnesium or magnesium alloy is in a molten state and/or during the cooling of the melt; however, this is not required. The one or more additives typically are added in a weight percent that is less than a weight percent of said magnesium or magnesium alloy. Typically, the magnesium or magnesium alloy constitutes about 50.1 wt % 99.9 wt % of the magnesium composite and all values and ranges therebetween. In one non-limiting aspect of the invention, the magnesium or magnesium alloy constitutes about 60 wt. % -95 wt. % of the magnesium composite, and typically the magnesium or magnesium alloy constitutes about 70 wt. % -90 wt. % of the magnesium composite. The one or more additives are typically added to the molten magnesium or magnesium alloy at a temperature that is less than the melting point of the one or more additives. The one or more additives generally have an average particle diameter size of at least about 0.1 microns, typically no more than about 500 microns (e.g., 0.1 microns, 0.1001 microns, 0.1002 microns . . . 499.9998 microns, 499.9999 microns, 500 microns) and including any value or range therebetween, more typically about 0.1 to 400 microns, and still more typically about 10 to 50 microns. During the process of mixing the one or more additives in the molten magnesium or magnesium alloy, the one or more additives are typically not caused to fully melt in the molten magnesium or magnesium alloy. As can be appreciated, the one or more additives can be added to the molten magnesium or magnesium alloy at a temperature that is greater than the melting point of the one or more additives. In such a method of forming the magnesium composite, the one or more additives form secondary metallic alloys with the magnesium and/or other metals in the magnesium alloy, said secondary metallic alloys having a melting point that is greater than the magnesium and/or other metals in the magnesium alloy. As the molten metal cools, these newly formed secondary metallic alloys begin to precipitate out of the molten metal and form the in situ phase to the matrix phase in the cooled and solid magnesium composite. After the mixing process is completed, the molten magnesium or magnesium alloy and the one or more additives that are mixed in the molten

magnesium or magnesium alloy are cooled to form a solid component. Generally, the temperature of the molten magnesium or magnesium alloy is at least about 10° C. less than the melting point of the additive added to the molten magnesium or magnesium alloy during the addition and mixing process, typically at least about 100° C. less than the melting point of the additive added to the molten magnesium or magnesium alloy during the addition and mixing process, more typically about 100° C.-1000° C. (and any value or range therebetween) less than the melting point of the additive added to the molten magnesium or magnesium alloy during the addition and mixing process; however, this is not required. The never melted particles and/or the newly formed secondary metallic alloys are referred to as in situ particle formation in the molten magnesium composite. Such a process can be used to achieve a specific galvanic corrosion rate in the entire magnesium composite and/or along the grain boundaries of the magnesium composite.

The invention adopts a feature that is usually a negative in traditional casting practices wherein a particle is formed during the melt processing that corrodes the alloy when exposed to conductive fluids and is imbedded in eutectic phases, the grain boundaries, and/or even within grains with precipitation hardening. This feature results in the ability to control where the galvanically-active phases are located in the final casting, as well as the surface area ratio of the in situ phase to the matrix phase, which enables the use of lower cathode phase loadings as compared to a powder metallurgical or alloyed composite to achieve the same dissolution rates. The in situ formed galvanic additives can be used to enhance mechanical properties of the magnesium composite such as ductility, tensile strength, and/or shear strength. The final magnesium composite can also be enhanced by heat treatment as well as deformation processing (such as extrusion, forging, or rolling) to further improve the strength of the final composite over the as-cast material; however, this is not required. The deformation processing can be used to achieve strengthening of the magnesium composite by reducing the grain size of the magnesium composite. Further enhancements, such as traditional alloy heat treatments (such as solutionizing, aging and/or cold working) can be used to enable control of dissolution rates through precipitation of more or less galvanically-active phases within the alloy microstructure while improving mechanical properties; however, this is not required. Because galvanic corrosion is driven by both the electro potential between the anode and cathode phase, as well as the exposed surface area of the two phases, the rate of corrosion can also be controlled through adjustment of the in situ formed particles size, while not increasing or decreasing the volume or weight fraction of the addition, and/or by changing the volume/weight fraction without changing the particle size. Achievement of in situ particle size control can be achieved by mechanical agitation of the melt, ultrasonic processing of the melt, controlling cooling rates, and/or by performing heat treatments. In situ particle size can also or alternatively be modified by secondary processing such as rolling, forging, extrusion and/or other deformation techniques.

In another non-limiting aspect of the invention, a cast structure can be made into almost any shape. During formation, the active galvanically-active in situ phases can be uniformly dispersed throughout the component and the grain or the grain boundary composition can be modified to achieve the desired dissolution rate. The galvanic corrosion can be engineered to affect only the grain boundaries and/or can affect the grains as well (based on composition); however, this is not required. This feature can be used to enable

fast dissolutions of high-strength lightweight alloy composites with significantly less active (cathode) in situ phases as compared to other processes.

In still another and/or alternative non-limiting aspect of the invention, ultrasonic processing can be used to control the size of the in situ formed galvanically-active phases; however, this is not required.

In yet another and/or alternative non-limiting aspect of the invention, the in situ formed particles can act as matrix strengtheners to further increase the tensile strength of the material compared to the base alloy without the additive; however, this is not required.

In still yet another and/or alternative non-limiting aspect of the invention, there is provided a method of controlling the dissolution properties of a metal selected from the class of magnesium and/or magnesium alloy comprising of the steps of a) melting the magnesium or magnesium alloy to a point above its solidus, b) introducing an additive material and/or phase to the magnesium or magnesium alloy in order to achieve in situ precipitation of galvanically-active intermetallic phases, and c) cooling the melt to a solid form. The additive material is generally added to the magnesium or magnesium alloy when the magnesium or magnesium alloy is in a molten state and at a temperature that is less than the melting point of the additive material. The galvanically-active intermetallic phases can be used to enhance the yield strength of the alloy; however, this is not required. The size of the in situ precipitated intermetallic phase can be controlled by a melt mixing technique and/or cooling rate; however, this is not required. The method can include the additional step of subjecting the magnesium composite to intermetallic precipitates to solutionizing of at least about 300° C. to improve tensile strength and/or improve ductility; however, this is not required. The solutionizing temperature is less than the melting point of the magnesium composite. Generally, the solutionizing temperature is less than 50° C.-200° C. (the melting point of the magnesium composite) and the time period of solutionizing is at least 0.1 hours. In one non-limiting aspect of the invention, the magnesium composite can be subjected to a solutionizing temperature for about 0.5-50 hours (e.g., 1-15 hours, etc.) at a temperature of 300° C.-620° C. (e.g., 300° C.-500° C., etc.). The method can include the additional step of subjecting the magnesium composite to intermetallic precipitates and to artificially age the magnesium composite at a temperature at least about 90° C. to improve the tensile strength; however, this is not required. The artificially aging process temperature is typically less than the solutionizing temperature and the time period of the artificially aging process temperature is typically at least 0.1 hours. Generally, the artificially aging process is less than 50° C.-400° C. (the solutionizing temperature). In one non-limiting aspect of the invention, the magnesium composite can be subjected to aging treatment for about 0.5-50 hours (e.g., 1-16 hours, etc.) at a temperature of 90° C.-300° C. (e.g., 100° C.-200° C.).

In another and/or alternative non-limiting aspect of the invention, there is provided a magnesium composite that is over 50 wt. % magnesium and about 0.05-35 wt. % nickel (and all values or ranges therebetween) is added to the magnesium or magnesium alloy to form intermetallic  $Mg_2Ni$  as a galvanically-active in situ precipitate. In one non-limiting arrangement, the magnesium composite includes about 0.05-23.5 wt. % nickel, 0.01-5 wt. % nickel, 3-7 wt. % nickel, 7-10 wt. % nickel, or 10-24.5 wt. % nickel. The nickel is added to the magnesium or magnesium alloy while the temperature of the molten magnesium or magnesium alloy is less than the melting point of the nickel. Throughout

the mixing process, the temperature of the molten magnesium or magnesium alloy is less than the melting point of the nickel. During the mixing process, solid particles of  $Mg_2Ni$  are formed. Once the mixing process is complete, the mixture of molten magnesium or magnesium alloy; solid particles of  $Mg_2Ni$ , and any unalloyed nickel particles are cooled and an in situ precipitate of solid particles of  $Mg_2Ni$  and any unalloyed nickel particles are formed in the solid magnesium or magnesium alloy. Generally, the temperature of the molten magnesium or magnesium alloy is at least about 200° C. less than the melting point of the nickel added to the molten magnesium or magnesium alloy during the addition and mixing process.

In still another and/or alternative non-limiting aspect of the invention, there is provided a magnesium composite that is over 50 wt. % magnesium and about 0.05-35 wt. % copper (and all values or ranges therebetween) is added to the magnesium or magnesium alloy to form intermetallic  $CuMg_2$  as the galvanically-active in situ precipitate. In one non-limiting arrangement, the magnesium composite includes about 0.01-5 wt. % copper, about 0.5-15 wt. % copper, about 15-35 wt. % copper, or about 0.01-20 wt. %. The copper is added to the magnesium or magnesium alloy while the temperature of the molten magnesium or magnesium alloy is less than the melting point of the copper. Throughout the mixing process, the temperature of the molten magnesium or magnesium alloy is less than the melting point of the copper. During the mixing process, solid particles of  $CuMg_2$  are formed. Once the mixing process is complete, the mixture of molten magnesium or magnesium alloy, solid particles of  $CuMg_2$ , and any unalloyed copper particles are cooled and an in situ precipitate of solid particles of  $CuMg_2$  and any unalloyed copper particles are formed in the solid magnesium or magnesium alloy. Generally, the temperature of the molten magnesium or magnesium alloy is at least about 200° C. less than the melting point of the copper added to the molten magnesium or magnesium alloy.

In yet another and/or alternative non-limiting aspect of the invention, there is provided a magnesium composite that is over 50 wt. % magnesium and about 0.05-20% by weight cobalt is added to the magnesium or magnesium alloy to form an intermetallic  $CoMg_2$  as the galvanically-active in situ precipitate. The cobalt is added to the magnesium or magnesium alloy while the temperature of the molten magnesium or magnesium alloy is less than the melting point of the cobalt. Throughout the mixing process, the temperature of the molten magnesium or magnesium alloy is less than the melting point of the cobalt. During the mixing process, solid particles of  $CoMg_2$  are formed. Once the mixing process is complete, the mixture of molten magnesium or magnesium alloy, solid particles of  $CoMg_2$ , and any unalloyed cobalt particles are cooled and an in situ precipitate of solid particles of  $CoMg_2$  and any unalloyed cobalt particles are formed in the solid magnesium or magnesium alloy. Generally, the temperature of the molten magnesium or magnesium alloy is at least about 200° C. less than the melting point of the cobalt added to the molten magnesium or magnesium alloy.

In yet another and/or alternative non-limiting aspect of the invention, there is provided a magnesium composite that is over 50 wt. % magnesium and cobalt is added to the magnesium or magnesium alloy which forms an intermetallic  $Mg_xCo$  as the galvanically-active particle in situ precipitate. The cobalt is added to the magnesium or magnesium alloy while the temperature of the molten magnesium or magnesium alloy is less than the melting point of the

cobalt. Throughout the mixing process, the temperature of the molten magnesium or magnesium alloy is less than the melting point of the cobalt. During the mixing process, solid particles of  $CoMg_x$  are formed. Once the mixing process is complete, the mixture of molten magnesium or magnesium alloy, solid particles of  $CoMg_x$ , and any unalloyed cobalt particles are cooled and an in situ precipitate of solid particles of  $CoMg_x$  and any unalloyed cobalt particles are formed in the solid magnesium or magnesium alloy. Generally, the temperature of the molten magnesium or magnesium alloy is at least about 200° C. less than the melting point of the cobalt added to the molten magnesium or magnesium alloy.

In still yet another and/or alternative non-limiting aspect of the invention, there is provided a magnesium composite that is over 50 wt. % magnesium and about 0.5-35% by weight of secondary metal (SM) is added to the magnesium or magnesium alloy to form a galvanically active intermetallic particle when compared to magnesium or a magnesium alloy in the remaining casting where the cooling rate between the liquidus to the solidus is faster than 1° C. per minute. The secondary metal is added to the magnesium or magnesium alloy while the temperature of the molten magnesium or magnesium alloy is less than the melting point of the secondary metal. Throughout the mixing process, the temperature of the molten magnesium or magnesium alloy is less than the melting point of the secondary metal. During the mixing process, solid particles of  $SMMg_x$  are formed. Once the mixing process is complete, the mixture of molten magnesium or magnesium alloy, solid particles of  $SMMg_x$ , and any unalloyed secondary metal particles are cooled and an in situ precipitate of solid particles of  $SMMg_x$  and any unalloyed secondary metal particles are formed in the solid magnesium or magnesium alloy. Generally, the temperature of the molten magnesium or magnesium alloy is at least about 200° C. less than the melting point of the secondary metal added to the molten magnesium or magnesium alloy. As can be appreciated, one or more secondary metals can be added to the molten magnesium or magnesium alloy.

In another and/or alternative non-limiting aspect of the invention, there is provided a magnesium composite that is over 50 wt. % magnesium and about 0.5-35% by weight of secondary metal (SM) is added to the magnesium or magnesium alloy to form a galvanically active intermetallic particle when compared to magnesium or a magnesium alloy in the remaining casting where the cooling rate between the liquidus to the solidus is slower than 1° C. per minute. The secondary metal is added to the magnesium or magnesium alloy while the temperature of the molten magnesium or magnesium alloy is less than the melting point of the secondary metal. Throughout the mixing process, the temperature of the molten magnesium or magnesium alloy is less than the melting point of the secondary metal. During the mixing process, solid particles of  $SMMg_x$  are formed. Once the mixing process is complete, the mixture of molten magnesium or magnesium alloy, solid particles of  $SMMg_x$ , and any unalloyed secondary metal particles are cooled and an in situ precipitate of solid particles of  $SMMg_x$  and any unalloyed secondary metal particles are formed in the solid magnesium or magnesium alloy. Generally, the temperature of the molten magnesium or magnesium alloy is at least about 200° C. less than the melting point of the secondary metal added to the molten magnesium or magnesium alloy. As can be appreciated, one or more secondary metals can be added to the molten magnesium or magnesium alloy.

In still another and/or alternative non-limiting aspect of the invention, there is provided a magnesium composite that

is over 50 wt. % magnesium and about 0.05-35 wt. % of secondary metal (SM) is added to the magnesium or magnesium alloy to form a galvanically-active intermetallic particle when compared to magnesium or a magnesium alloy in the remaining casting where the cooling rate between the liquidus to the solidus is faster than 0.01° C. per min and slower than 1° C. per minute. The secondary metal is added to the magnesium or magnesium alloy while the temperature of the molten magnesium or magnesium alloy is less than the melting point of the secondary metal. Throughout the mixing process, the temperature of the molten magnesium or magnesium alloy is less than the melting point of the secondary metal. During the mixing process, solid particles of  $SMMg_x$  are formed. Once the mixing process is complete, the mixture of molten magnesium or magnesium alloy, solid particles of  $SMMg_x$  and any unalloyed secondary metal particles are cooled and an in situ precipitate of solid particles of  $SMMg_x$  and any unalloyed secondary metal particles are formed in the solid magnesium or magnesium alloy. Generally, the temperature of the molten magnesium or magnesium alloy is at least about 200° C. less than the melting point of the secondary metal added to the molten magnesium or magnesium alloy. As can be appreciated, one or more secondary metals can be added to the molten magnesium or magnesium alloy.

In yet another and/or alternative non-limiting aspect of the invention, there is provided a magnesium composite that is over 50 wt. % magnesium and about 0.05-35 wt. % of secondary metal (SM) is added to the magnesium or magnesium alloy to form a galvanically-active intermetallic particle when compared to magnesium or a magnesium alloy in the remaining casting where the cooling rate between the liquidus to the solidus is faster than 10° C. per minute. The secondary metal is added to the magnesium or magnesium alloy while the temperature of the molten magnesium or magnesium alloy is less than the melting point of the secondary metal. Throughout the mixing process, the temperature of the molten magnesium or magnesium alloy is less than the melting point of the secondary metal. During the mixing process, solid particles of  $SMMg_x$  were formed. Once the mixing process was completed, the mixture of molten magnesium or magnesium alloy, solid particles of  $SMMg_x$ , and any unalloyed secondary metal particles are cooled and an in situ precipitate of solid particles of  $SMMg_x$  and any unalloyed secondary metal particles are formed in the solid magnesium or magnesium alloy. Generally, the temperature of the molten magnesium or magnesium alloy is at least about 200° C. less than the melting point of the secondary metal added to the molten magnesium or magnesium alloy. As can be appreciated, one or more secondary metals can be added to the molten magnesium or magnesium alloy.

In still yet another and/or alternative non-limiting aspect of the invention, there is provided magnesium composite that is over 50 wt. % magnesium and about 0.5-35 wt. % of secondary metal (SM) is added to the magnesium or magnesium alloy to form a galvanically-active intermetallic particle when compared to magnesium or a magnesium alloy in the remaining casting where the cooling rate between the liquidus to the solidus is slower than 10° C. per minute. The secondary metal is added to the magnesium or magnesium alloy while the temperature of the molten magnesium or magnesium alloy is less than the melting point of the secondary metal. Throughout the mixing process, the temperature of the molten magnesium or magnesium alloy is less than the melting point of the secondary metal. During the mixing process, solid particles of  $SMMg_x$  are formed.

Once the mixing process is complete, the mixture of molten magnesium or magnesium alloy, solid particles of  $SMMg_x$ , and any unalloyed secondary metal particles are cooled and an in situ precipitate of solid particles of  $SMMg_x$  and any unalloyed secondary metal particles are formed in the solid magnesium or magnesium alloy. Generally, the temperature of the molten magnesium or magnesium alloy is at least about 200° C. less than the melting point of the secondary metal added to the molten magnesium or magnesium alloy.

10 As can be appreciated, one or more secondary metals can be added to the molten magnesium or magnesium alloy.

In another and/or alternative non-limiting aspect of the invention, there is provided a magnesium alloy that includes over 50 wt. % magnesium and includes at least one metal selected from the group consisting of aluminum in an amount of about 0.5-10 wt. %, zinc in amount of about 0.05-6 wt. %, zirconium in an amount of about 0.01-3 wt. %, and/or manganese in an amount of about 0.15-2 wt. %. In one non-limiting formulation, the magnesium alloy that includes over 50 wt. % magnesium and includes at least one metal selected from the group consisting of zinc in amount of about 0.05-6 wt. %, zirconium in an amount of about 0.05-3 wt. %, manganese in an amount of about 0.05-0.25 wt. %, boron in an amount of about 0.0002-0.04 wt. %, and bismuth in an amount of about 0.4-0.7 wt. %. The magnesium alloy can then be heated to a molten state and one or more secondary metal (SM) (e.g., copper, nickel, cobalt, titanium, silicon, iron, etc.) can be added to the molten magnesium alloy which forms an intermetallic galvanically-active particle in situ precipitate. The galvanically-active particle can be  $SMMg_x$ ,  $SMAl_x$ ,  $SMZn_x$ ,  $SMZr_x$ ,  $SMMn_x$ ,  $SMB_x$ ,  $SMBi_x$ , SM in combination with anyone of B, Bi, Mg, Al, Zn, Zr, and Mn.

In still another and/or alternative non-limiting aspect of the invention, there is provided a magnesium composite that is over 50 wt. % magnesium and at least one metal selected from the group consisting of zinc in an amount of about 0.05-6 wt. %, zirconium in amount of about 0.05-3 wt. %, manganese in an amount of about 0.05-0.25 wt. %, boron in an amount of about 0.0002-0.04 wt. %, and/or bismuth in an amount of about 0.4-0.7 wt. % is added to the magnesium or magnesium alloy to form a galvanically-active intermetallic particle in the magnesium or magnesium alloy. The magnesium alloy can then be heated to a molten state and one or more secondary metal (SM) (e.g., copper, nickel, cobalt, titanium, iron, etc.) can be added to the molten magnesium alloy which forms an intermetallic galvanically-active particle in situ precipitate. The galvanically-active particle can be  $SMMg_x$ ,  $SMZn_x$ ,  $SMZr_x$ ,  $SMMn_x$ ,  $SMB_x$ ,  $SMBi_x$ , SM in combination with anyone of Mg, Zn, Zr, Mn, B and/or Bi.

In yet another and/or alternative non-limiting aspect of the invention, there is provided a magnesium or magnesium alloy that is over 50 wt. % magnesium and nickel in an amount of about 0.01-5 wt. % is added to the magnesium or magnesium alloy to form a galvanically-active intermetallic particle in the magnesium or magnesium alloy. The nickel is added to the magnesium or magnesium alloy while the temperature of the molten magnesium or magnesium alloy is less than the melting point of the nickel. Throughout the mixing process, the temperature of the molten magnesium or magnesium alloy is less than the melting point of the nickel. During the mixing process, solid particles of  $Mg_2Ni$  are formed. Once the mixing process is complete, the mixture of molten magnesium or magnesium alloy, solid particles of  $Mg_2Ni$ , and any unalloyed nickel particles are cooled and an in situ precipitate of solid particles of  $Mg_2Ni$  and any unalloyed nickel particles are formed in the solid magne-



## 11

C. less than the melting point of the copper added to the molten magnesium or magnesium alloy during the addition and mixing process.

In still another and/or alternative non-limiting aspect of the invention, there is provided a magnesium composite that is over 50 wt. % magnesium and includes copper in an amount of about 0.01-20 wt. % is added to the magnesium or magnesium alloy to form a galvanically-active intermetallic particle in the magnesium or magnesium alloy. The copper is added to the magnesium or magnesium alloy while the temperature of the molten magnesium or magnesium alloy is less than the melting point of the copper. Throughout the mixing process, the temperature of the molten magnesium or magnesium alloy is less than the melting point of the copper. During the mixing process, solid particles of  $Mg_2Cu$  are formed. Once the mixing process is complete, the mixture of molten magnesium or magnesium alloy, solid particles of  $Mg_2Cu$ , and any unalloyed nickel particles are cooled and an in situ precipitate of solid particles of  $Mg_2Cu$  and any unalloyed copper particles are formed in the solid magnesium or magnesium alloy. Generally, the temperature of the molten magnesium or magnesium alloy is at least about 200° C. less than the melting point of the copper added to the molten magnesium or magnesium alloy during the addition and mixing process.

In yet another and/or alternative non-limiting aspect of the invention, there is provided a magnesium composite that is subjected to heat treatments such as solutionizing, aging and/or cold working to be used to control dissolution rates though precipitation of more or less galvanically-active phases within the alloy microstructure while improving mechanical properties. The aging process (when used) can be for at least about 1 hour, for about 1-50 hours, for about 1-20 hours, or for about 8-20 hours. The solutionizing (when used) can be for at least about 1 hour, for about 1-50 hours, for about 1-20 hours, or for about 8-20 hours.

In still yet another and/or alternative non-limiting aspect of the invention, there is provided a method for controlling the dissolution rate of the magnesium composite wherein the magnesium content is at least about 75% and nickel is added to form in situ precipitation of at least 0.05 wt. %  $MgNi_2$  with the magnesium or magnesium alloy and solutionizing the resultant metal at a temperature within a range of 100-500° C. for a period of 0.25-50 hours, the magnesium composite being characterized by higher dissolution rates than metal without nickel additions subjected to the said aging treatment.

In another and/or alternative non-limiting aspect of the invention, there is provided a method for improving the physical properties of the magnesium composite wherein the magnesium content is at least about 85% and nickel is added to form in situ precipitation of at least 0.05 wt. %  $MgNi_2$  with the magnesium or magnesium alloy and solutionizing the resultant metal at a temperature at about 100-500° C. for a period of 0.25-50 hours, the magnesium composite being characterized by higher tensile and yield strengths than magnesium base alloys of the same composition, but not including the amount of nickel.

In still another and/or alternative non-limiting aspect of the invention, there is provided a method for controlling the dissolution rate of the magnesium composite wherein the magnesium content in the alloy is at least about 75% and copper is added to form in situ precipitation of at least about 0.05 wt. %  $MgCu_2$  with the magnesium or magnesium alloy and solutionizing the resultant metal at a temperature within a range of 100-500° C. for a period of 0.25-50 hours, the

## 12

magnesium composite being characterized by higher dissolution rates than metal without copper additions subjected to the said aging treatment.

In yet another and/or alternative non-limiting aspect of the invention, there is provided a method for improving the physical properties of the magnesium composite wherein the total content of magnesium in the magnesium or magnesium alloy is at least about 85 wt. % and copper is added to form in situ precipitation of at least 0.05 wt. %  $MgCu_2$  with the magnesium or magnesium composite and solutionizing the resultant metal at a temperature of about 100-500° C. for a period of 0.25-50 hours, the magnesium composite is characterized by higher tensile and yield strengths than magnesium base alloys of the same composition, but not including the amount of copper.

In still yet another and/or alternative non-limiting aspect of the invention, there is provided a magnesium composite for use as a dissolvable ball or frac ball in hydraulic fracturing and well drilling.

In another and/or alternative non-limiting aspect of the invention, there is provided a magnesium composite for use as a dissolvable tool for use in well drilling and hydraulic control as well as hydraulic fracturing.

In still another and/or alternative non-limiting aspect of the invention, there is provided a magnesium composite that includes secondary institute formed reinforcements that are not galvanically-active to the magnesium or magnesium alloy matrix to increase the mechanical properties of the magnesium composite. The secondary institute formed reinforcements include a  $Mg_2Si$  phase as the in situ formed reinforcement.

In yet another and/or alternative non-limiting aspect of the invention, there is provided a magnesium composite that is subjected to a faster cooling rate from the liquidus to the solidus point to create smaller in situ formed particles.

In still yet another and/or alternative non-limiting aspect of the invention, there is provided a magnesium composite that is subjected to a slower cooling rate from the liquidus to the solidus point to create larger in situ formed particles.

In yet another and/or alternative non-limiting aspect of the invention, there is provided a magnesium composite that is subjected to heat treatments such as solutionizing, aging and/or cold working to be used to control dissolution rates though precipitation of more or less galvanically-active phases within the alloy microstructure while improving mechanical properties. The aging process (when used) can be for at least about 1 hour, for about 1-50 hours, for about 1-20 hours, or for about 8-20 hours. The solutionizing (when used) can be for at least about 1 hour, for about 1-50 hours, for about 1-20 hours, or for about 8-20 hours.

In still yet another and/or alternative non-limiting aspect of the invention, there is provided a method for controlling the dissolution rate of the magnesium composite wherein the magnesium content is at least about 75% and nickel is added to form in situ precipitation of at least 0.05 wt. %  $MgNi_2$  with the magnesium or magnesium alloy and solutionizing the resultant metal at a temperature within a range of 100-500° C. for a period of 0.25-50 hours, the magnesium composite being characterized by higher dissolution rates than metal without nickel additions subjected to the said aging treatment.

In another and/or alternative non-limiting aspect of the invention, there is provided a method for improving the physical properties of the magnesium composite wherein the magnesium content is at least about 85% and nickel is added to form in situ precipitation of at least 0.05 wt. %  $MgNi_2$  with the magnesium or magnesium alloy and solutionizing

## 13

the resultant metal at a temperature at about 100-500° C. for a period of 0.25-50 hours, the magnesium composite being characterized by higher tensile and yield strengths than magnesium base alloys of the same composition, but not including the amount of nickel.

In still another and/or alternative non-limiting aspect of the invention, there is provided a method for controlling the dissolution rate of the magnesium composite wherein the magnesium content in the alloy is at least about 75% and copper is added to form in situ precipitation of at least about 0.05 wt. %  $MgCu_2$  with the magnesium or magnesium alloy and solutionizing the resultant metal at a temperature within a range of 100-500° C. for a period of 0.25-50 hours, the magnesium composite being characterized by higher dissolution rates than metal without copper additions subjected to the said aging treatment.

In yet another and/or alternative non-limiting aspect of the invention, there is provided a method for improving the physical properties of the magnesium composite wherein the total content of magnesium in the magnesium or magnesium alloy is at least about 85 wt. % and copper is added to form in situ precipitation of at least 0.05 wt. %  $MgCu_2$  with the magnesium or magnesium composite and solutionizing the resultant metal at a temperature of about 100-500° C. for a period of 0.25-50 hours, the magnesium composite is characterized by higher tensile and yield strengths than magnesium base alloys of the same composition, but not including the amount of copper.

In still yet another and/or alternative non-limiting aspect of the invention, there is provided a magnesium composite for use as a dissolvable ball or frac ball in hydraulic fracturing and well drilling.

In another and/or alternative non-limiting aspect of the invention, there is provided a magnesium composite for use as a dissolvable tool for use in well drilling and hydraulic control as well as hydraulic fracturing.

In still another and/or alternative non-limiting aspect of the invention, there is provided a magnesium composite that includes secondary institute formed reinforcements that are not galvanically-active to the magnesium or magnesium alloy matrix to increase the mechanical properties of the magnesium composite. The secondary institute formed reinforcements include a  $Mg_2Si$  phase as the in situ formed reinforcement.

In yet another and/or alternative non-limiting aspect of the invention, there is provided a magnesium composite that is subjected to a faster cooling rate from the liquidus to the solidus point to create smaller in situ formed particles.

In still yet another and/or alternative non-limiting aspect of the invention, there is provided a magnesium composite that is subjected to a slower cooling rate from the liquidus to the solidus point to create larger in situ formed particles.

In another and/or alternative non-limiting aspect of the invention, there is provided a magnesium composite that is subjected to mechanical agitation during the cooling rate from the liquidus to the solidus point to create smaller in situ formed particles.

In another and/or alternative non-limiting aspect of the invention, there is provided a magnesium composite that is subjected to mechanical agitation during the cooling rate from the liquidus to the solidus point to create smaller in situ formed particles.

In still another and/or alternative non-limiting aspect of the invention, there is provided a magnesium composite that is subjected to chemical agitation during the cooling rate from the liquidus to the solidus point to create smaller in situ formed particles.

## 14

In yet another and/or alternative non-limiting aspect of the invention, there is provided a magnesium composite that is subjected to ultrasonic agitation during the cooling rate from the liquidus to the solidus point to create smaller in situ formed particles.

In still yet another and/or alternative non-limiting aspect of the invention, there is provided a magnesium composite that is subjected to deformation or extrusion to further improve dispersion of the in situ formed particles.

In another and/or alternative non-limiting aspect of the invention, there is provided a method for forming a novel magnesium composite including the steps of a) selecting an AZ91D magnesium alloy having 9 wt. % aluminum, 1 wt. % zinc and 90 wt. % magnesium, b) melting the AZ91D magnesium alloy to a temperature above 800° C., c) adding up to about 7 wt. % nickel to the melted AZ91D magnesium alloy at a temperature that is less than the melting point of nickel, d) mixing the nickel with the melted AZ91D magnesium alloy and dispersing the nickel in the melted alloy

15 using chemical mixing agents while maintaining the temperature below the melting point of nickel, and e) cooling and casting the melted mixture in a steel mold. The cast material has a tensile strength of about 14 ksi, and an elongation of about 3% and a shear strength of 11 ksi. The cast material has a dissolve rate of about 75 mg/cm<sup>2</sup>-min in a 3% KCl solution at 90° C. The cast material dissolves at a rate of 1 mg/cm<sup>2</sup>-hr in a 3% KCl solution at 21° C. The cast material dissolves at a rate of 325 mg/cm<sup>2</sup>-hr. in a 3% KCl solution at 90° C. The cast material can be subjected to

20 extrusion with a 11:1 reduction area. The extruded cast material exhibits a tensile strength of 40 ksi, and an elongation to failure of 12%. The extruded cast material dissolves at a rate of 0.8 mg/cm<sup>2</sup>-min in a 3% KCl solution at 20° C. The extruded cast material dissolves at a rate of 100 mg/cm<sup>2</sup>-hr. in a 3% KCl solution at 90° C. The extruded cast material can be subjected to an artificial T5 age treatment of

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 968

## 15

a 3% KCl solution at 90° C. The cast material dissolves at a rate of 0.5 mg/cm<sup>2</sup>-hr. in a 3% KCl solution at 21° C. The cast material dissolves at a rate of 325 mg/cm<sup>2</sup>-hr. in a 3% KCl solution at 90° C. The cast material was then subjected to extrusion with a 20:1 reduction area. The extruded cast material exhibits a tensile yield strength of 35 ksi, and an elongation to failure of 12%. The extruded cast material dissolves at a rate of 0.8 mg/cm<sup>2</sup>-min in a 3% KCl solution at 20° C. The extruded cast material dissolves at a rate of 50 mg/cm<sup>2</sup>-hr in a 3% KCl solution at 90° C. The extruded cast material can be subjected to an artificial T5 age treatment of 16 hours between 100° C.-200° C. The aged extruded cast material exhibits a tensile strength of 48 ksi, an elongation to failure of 5%, and a shear strength of 25 ksi.

In still another and/or alternative non-limiting aspect of the invention, there is provided a method for forming a novel magnesium composite including the steps of a) selecting an AZ91D magnesium alloy having about 9 wt. % aluminum, 1 wt. % zinc and 90 wt. % magnesium, b) melting the AZ91D magnesium alloy to a temperature above 800° C., c) adding about 10 wt. % copper to the melted AZ91D magnesium alloy at a temperature that is less than the melting point of copper, d) dispersing the copper in the melted AZ91D magnesium alloy using chemical mixing agents at a temperature that is less than the melting point of copper, and e) cooling casting the melted mixture in a steel mold. The cast material exhibits a tensile strength of about 14 ksi, an elongation of about 3%, and shear strength of 11 ksi. The cast material dissolves at a rate of about 50 mg/cm<sup>2</sup>-hr. in a 3% KCl solution at 90° C. The cast material dissolves at a rate of 0.6 mg/cm<sup>2</sup>-hr. in a 3% KCl solution at 21° C. The cast material can be subjected to an artificial T5 age treatment for about 16 hours at a temperature of 100-200° C. The aged cast material exhibits a tensile strength of 50 ksi, an elongation to failure of 5%, and a shear strength of 25 ksi. The aged cast material dissolved at a rate of 40 mg/cm<sup>2</sup>-hr in 3% KCl solution at 90° C. and 0.5 mg/cm<sup>2</sup>-hr in 3% KCl solution at 20° C.

These and other objects, features and advantages of the present invention will become apparent in light of the following detailed description of preferred embodiments thereof, as illustrated in the accompanying drawings.

## BRIEF DESCRIPTION OF THE DRAWINGS

FIGS. 1-3 show a typical cast microstructure with galvanically-active in situ formed intermetallic phase wetted to the magnesium matrix; and,

FIG. 4 shows a typical phase diagram to create in situ formed particles of an intermetallic Mg<sub>x</sub>(M) where M is any element on the periodic table or any compound in a magnesium matrix and wherein M has a melting point that is greater than the melting point of Mg.

## DETAILED DESCRIPTION OF THE INVENTION

The present invention is directed to a novel magnesium composite that can be used to form a castable, moldable, or extrudable component. The magnesium composite includes at least 50 wt. % magnesium. Generally, the magnesium composite includes over 50 wt. % magnesium and less than about 99.5 wt. % magnesium and all values and ranges therebetween. One or more additives are added to a magnesium or magnesium alloy to form the novel magnesium composite of the present invention. The one or more additives can be selected and used in quantities so that galvanically-

## 16

active intermetallic or insoluble precipitates form in the magnesium or magnesium alloy while the magnesium or magnesium alloy is in a molten state and/or during the cooling of the melt; however, this is not required. The one or more additives are added to the molten magnesium or magnesium alloy at a temperature that is less than the melting point of the one or more additives. During the process of mixing the one or more additives in the molten magnesium or magnesium alloy, the one or more additives are not caused to fully melt in the molten magnesium or magnesium alloy. After the mixing process is completed, the molten magnesium or magnesium alloy and the one or more additives that are mixed in the molten magnesium or magnesium alloy are cooled to form a solid component. Such a formation in the melt is called in situ particle formation as illustrated in FIGS. 1-3. Such a process can be used to achieve a specific galvanic corrosion rate in the entire magnesium composite and/or along the grain boundaries of the magnesium composite. This feature results in the ability to control where the galvanically-active phases are located in the final casting, as well as the surface area ratio of the in situ phase to the matrix phase, which enables the use of lower cathode phase loadings as compared to a powder metallurgical or alloyed composite to achieve the same dissolution rates. The in situ formed galvanic additives can be used to enhance mechanical properties of the magnesium composite such as ductility, tensile strength, and/or shear strength. The final magnesium composite can also be enhanced by heat treatment as well as deformation processing (such as extrusion, forging, or rolling) to further improve the strength of the final composite over the as-cast material; however, this is not required. The deformation processing can be used to achieve strengthening of the magnesium composite by reducing the grain size of the magnesium composite. Further enhancements, such as traditional alloy heat treatments (such as solutionizing, aging and/or cold working) can be used to enable control of dissolution rates through precipitation of more or less galvanically-active phases within the alloy microstructure while improving mechanical properties; however, this is not required. Because galvanic corrosion is driven by both the electro potential between the anode and cathode phase, as well as the exposed surface area of the two phases, the rate of corrosion can also be controlled through adjustment of the in situ formed particles size, while not increasing or decreasing the volume or weight fraction of the addition, and/or by changing the volume/weight fraction without changing the particle size. Achievement of in situ particle size control can be achieved by mechanical agitation of the melt, ultrasonic processing of the melt, controlling cooling rates, and/or by performing heat treatments. In situ particle size can also or alternatively be modified by secondary processing such as rolling, forging, extrusion and/or other deformation techniques. A smaller particle size can be used to increase the dissolution rate of the magnesium composite. An increase in the weight percent of the in situ formed particles or phases in the magnesium composite can also or alternatively be used to increase the dissolution rate of the magnesium composite. A phase diagram for forming in situ formed particles or phases in the magnesium composite is illustrated in FIG. 4.

In accordance with the present invention, a novel magnesium composite is produced by casting a magnesium metal or magnesium alloy with at least one component to form a galvanically-active phase with another component in the chemistry that forms a discrete phase that is insoluble at the use temperature of the dissolvable component. The in

situ formed particles and phases have a different galvanic potential from the remaining magnesium metal or magnesium alloy. The in situ formed particles or phases are uniformly dispersed through the matrix metal or metal alloy using techniques such as thixomolding, stir casting, mechanical agitation, chemical agitation, electrowetting, ultrasonic dispersion, and/or combinations of these methods. Due to the particles being formed in situ to the melt, such particles generally have excellent wetting to the matrix phase and can be found at grain boundaries or as continuous dendritic phases throughout the component depending on alloy composition and the phase diagram. Because the alloys form galvanic intermetallic particles where the intermetallic phase is insoluble to the matrix at use temperatures, once the material is below the solidus temperature, no further dispersing or size control is necessary in the component. This feature also allows for further grain refinement of the final alloy through traditional deformation processing to increase tensile strength, elongation to failure, and other properties in the alloy system that are not achievable without the use of insoluble particle additions. Because the ratio of in situ formed phases in the material is generally constant and the grain boundary to grain surface area is typically consistent even after deformation processing and heat treatment of the composite, the corrosion rate of such composites remains very similar after mechanical processing.

## EXAMPLE I

An AZ91D magnesium alloy having 9 wt. % aluminum, 1 wt. % zinc and 90 wt. % magnesium was melted to above 800° C. and at least 200° C. below the melting point of nickel. About 7 wt. % of nickel was added to the melt and dispersed. The melt was cast into a steel mold. The cast material exhibited a tensile strength of about 14 ksi, an elongation of about 3%, and shear strength of 11 ksi. The cast material dissolved at a rate of about 75 mg/cm<sup>2</sup>-min in a 3% KCl solution at 90° C. The material dissolved at a rate of 1 mg/cm<sup>2</sup>-hr in a 3% KCl solution at 21° C. The material dissolved at a rate of 325 mg/cm<sup>2</sup>-hr. in a 3% KCl solution at 90° C.

## EXAMPLE 2

The composite in Example 1 was subjected to extrusion with an 11:1 reduction area. The material exhibited a tensile yield strength of 45 ksi, an Ultimate tensile strength of 50 ksi and an elongation to failure of 8%. The material has a dissolve rate of 0.8 mg/cm<sup>2</sup>-min. in a 3% KCl solution at 20° C. The material dissolved at a rate of 100 mg/cm<sup>2</sup>-hr. in a 3% KCl solution at 90° C.

## EXAMPLE 3

The alloy in Example 2 was subjected to an artificial T5 age treatment of 16 hours from 100° C.-200° C. The alloy exhibited a tensile strength of 48 ksi and elongation to failure of 5% and a shear strength of 25 ksi. The material dissolved at a rate of 110 mg/cm<sup>2</sup>-hr. in 3% KCl solution at 90° C. and 1 mg/cm<sup>2</sup>-hr. in 3% KCl solution at 20° C.

## EXAMPLE 4

The alloy in Example 1 was subjected to a solutionizing treatment T4 of 18 hours from 400° C.-500° C. and then an artificial T6 aging treatment of 16 hours from 100° C.-200° C. The alloy exhibited a tensile strength of 34 ksi and

elongation to failure of 11% and a shear strength of 18 ksi. The material dissolved at a rate of 84 mg/cm<sup>2</sup>-hr. in 3% KCl solution at 90° C. and 0.8 mg/cm<sup>2</sup>-hr. in 3% KCl solution at 20° C.

## EXAMPLE 5

An AZ91D magnesium alloy having 9 wt. % aluminum, 1 wt. % zinc and 90 wt. % magnesium was melted to above 800° C. and at least 200° C. below the melting point of copper. About 10 wt. % of copper alloyed to the melt and dispersed. The melt was cast into a steel mold. The cast material exhibited a tensile yield strength of about 14 ksi, an elongation of about 3%, and shear strength of 11 ksi. The cast material dissolved at a rate of about 50 mg/cm<sup>2</sup>-hr. in a 3% KCl solution at 90° C. The material dissolved at a rate of 0.6 mg/cm<sup>2</sup>-hr. in a 3% KCl solution at 21° C.

## EXAMPLE 6

The alloy in Example 5 was subjected to an artificial T5 aging treatment of 16 hours from 100° C.-200° C. the alloy exhibited a tensile strength of 50 ksi and elongation to failure of 5% and a shear strength of 25 ksi. The material dissolved at a rate of 40 mg/cm<sup>2</sup>-hr. in 3% KCl solution at 90° C. and 0.5 mg/cm<sup>2</sup>-hr. in 3% KCl solution at 20° C.

It will thus be seen that the objects set forth above, among those made apparent from the preceding description, are efficiently attained, and since certain changes may be made in the constructions set forth without departing from the spirit and scope of the invention, it is intended that all matter contained in the above description and shown in the accompanying drawings shall be interpreted as illustrative and not in a limiting sense. The invention has been described with reference to preferred and alternate embodiments. Modifications and alterations will become apparent to those skilled in the art upon reading and understanding the detailed discussion of the invention provided herein. This invention is intended to include all such modifications and alterations insofar as they come within the scope of the present invention. It is also to be understood that the following claims are intended to cover all of the generic and specific features of the invention herein described and all statements of the scope of the invention, which, as a matter of language, might be said to fall there between. The invention has been described with reference to the preferred embodiments. These and other modifications of the preferred embodiments as well as other embodiments of the invention will be obvious from the disclosure herein, whereby the foregoing descriptive matter is to be interpreted merely as illustrative of the invention and not as a limitation. It is intended to include all such modifications and alterations insofar as they come within the scope of the appended claims.

What is claimed:

1. A downhole well component at least partially formed of a dissolvable magnesium cast material, said dissolvable magnesium cast material comprising a mixture of magnesium and additive material or a mixture of magnesium alloy and additive material, said additive material includes i) copper wherein said copper constitutes 0.1-35 wt. % of said dissolvable magnesium cast material, ii) nickel wherein said nickel constitutes 0.1-24.5 wt. % of said dissolvable magnesium cast material, and/or iii) cobalt wherein said cobalt constitutes 0.1-20 wt. % of said dissolvable magnesium cast material, said dissolvable magnesium cast material includes galvanically-active in situ precipitate, said galvanically-active in situ precipitate includes said additive material, said

## 19

dissolvable magnesium cast material has a dissolution rate of at least 40 mg/cm<sup>2</sup>/hr. in 3 wt. % KCl water mixture at 90° C., said downhole well component includes one or more components selected from the group consisting of a sleeve, a ball, a frac ball, a hydraulic actuating tooling, a tube, a valve, a valve component, and a plug.

2. The downhole well component as defined in claim 1, wherein said dissolvable magnesium cast material includes no more than 10 wt. % aluminum.

3. The downhole well component as defined in claim 1, wherein said dissolvable magnesium cast material has a dissolution rate of at least 75 mg/cm<sup>2</sup>/hr. in 3 wt. % KCl water mixture at 90° C.

4. The downhole well component as defined in claim 1, wherein said dissolvable magnesium cast material includes at least 85 wt. % magnesium.

5. The downhole well component as defined in claim 1, wherein said dissolvable magnesium cast material has a dissolution rate of 40-325 mg/cm<sup>2</sup>/hr. in 3 wt. % KCl water mixture at 90° C.

6. The downhole well component as defined in claim 2, wherein said dissolvable magnesium cast material has a dissolution rate of 40-325 mg/cm<sup>2</sup>/hr. in 3 wt. % KCl water mixture at 90° C.

7. The downhole well component as defined in claim 4, wherein said dissolvable magnesium cast material has a dissolution rate of 40-325 mg/cm<sup>2</sup>/hr. in 3 wt. % KCl water mixture at 90° C.

8. The downhole well component as defined in claim 2, wherein said dissolvable magnesium cast material includes at least 85 wt. % magnesium.

9. The downhole well component as defined in claim 3, wherein said dissolvable magnesium cast material includes at least 85 wt. % magnesium.

10. The downhole well component as defined in claim 5, wherein said dissolvable magnesium cast material includes at least 85 wt. % magnesium.

11. The downhole well component as defined in claim 6, wherein said dissolvable magnesium cast material includes at least 85 wt. % magnesium.

12. The downhole well component as defined in claim 8, wherein said dissolvable magnesium cast material has a dissolution rate of at least 75 mg/cm<sup>2</sup>/hr. in 3 wt. % KCl water mixture at 90° C.

13. The downhole well component as defined in claim 2, wherein said dissolvable magnesium cast material includes at least 50 wt. % magnesium.

14. The downhole well component as defined in claim 13, wherein said dissolvable magnesium cast material has a dissolution rate of at least 75 mg/cm<sup>2</sup>/hr. in 3 wt. % KCl water mixture at 90° C.

15. The downhole well component as defined in claim 1, wherein said magnesium alloy includes over 50 wt. % magnesium and one or more metals selected from the group consisting of aluminum, boron, bismuth, zinc, zirconium, and manganese.

16. The downhole well component as defined in claim 13, wherein said magnesium alloy includes over 50 wt. % magnesium and one or more metals selected from the group consisting of aluminum, boron, bismuth, zinc, zirconium, and manganese.

17. The downhole well component as defined in claim 14, wherein said magnesium alloy includes over 50 wt. % magnesium and one or more metals selected from the group consisting of aluminum, boron, bismuth, zinc, zirconium, and manganese.

## 20

18. The downhole well component as defined in claim 17, wherein said magnesium alloy includes over 50 wt. % magnesium and one or more metals selected from the group consisting of aluminum in an amount of 0.5-10 wt. %, zinc in an amount of 0.1-6 wt. %, zirconium in an amount of 0.01-3 wt. %, manganese in an amount of 0.15-2 wt. %, boron in an amount of 0.0002-0.04 wt. %, and bismuth in an amount of 0.4-0.7 wt. %.

19. The downhole well component as defined in claim 17, wherein said magnesium alloy includes over 50 wt. % magnesium and one or more metals selected from the group consisting of aluminum in an amount of 0.5-10 wt. %, zinc in an amount of 0.1-3 wt. %, zirconium in an amount of 0.01-1 wt. %, manganese in an amount of 0.15-2 wt. %, boron in an amount of 0.0002-0.04 wt. %, and bismuth in amount of 0.4-0.7 wt. %.

20. The downhole well component as defined in claim 17, wherein said magnesium alloy includes at least 85 wt. % magnesium and one or more metals selected from the group consisting of 0.5-10 wt. % aluminum, 0.05-6 wt. % zinc, 0.01-3 wt. % zirconium, and 0.15-2 wt. % manganese.

21. The downhole well component as defined in claim 4, wherein said magnesium alloy includes at least 85 wt. % magnesium and one or more metals selected from the group consisting of 0.5-10 wt. % aluminum, 0.05-6 wt. % zinc, 0.01-3 wt. % zirconium, and 0.15-2 wt. % manganese.

22. The downhole well component as defined in claim 9, wherein said magnesium alloy includes at least 85 wt. % magnesium and one or more metals selected from the group consisting of 0.5-10 wt. % aluminum, 0.05-6 wt. % zinc, 0.01-3 wt. % zirconium, and 0.15-2 wt. % manganese.

23. The downhole well component as defined in claim 12, wherein said magnesium alloy includes at least 85 wt. % magnesium and one or more metals selected from the group consisting of 0.5-10 wt. % aluminum, 0.05-6 wt. % zinc, 0.01-3 wt. % zirconium, and 0.15-2 wt. % manganese.

24. The downhole well component as defined in claim 17, wherein said magnesium alloy comprises greater than 50 wt. % magnesium and one or more metals selected from the group consisting of 0.5-10 wt. % aluminum, 0.1-2 wt. % zinc, 0.01-1 wt. % zirconium, and 0.15-2 wt. % manganese.

25. The downhole well component as defined in claim 17, wherein said magnesium alloy comprises greater than 50 wt. % magnesium and one or more metals selected from the group consisting of 0.1-3 wt. % zinc, 0.05-1 wt. % zirconium, 0.05-0.25 wt. % manganese, 0.0002-0.04 wt. % boron, and 0.4-0.7 wt. % bismuth.

26. The downhole well component as defined in claim 17, wherein said magnesium alloy comprises 60-95 wt. % magnesium, 0.5-10 wt. % aluminum, 0.05-6 wt. % zinc, and 0.15-2 wt. % manganese.

27. The downhole well component as defined in claim 17, wherein said magnesium alloy includes 60-95 wt. % magnesium and 0.01-1 wt. % zirconium.

28. The downhole well component as defined in claim 17, wherein said magnesium alloy includes 60-95 wt. % magnesium, 0.05-6 wt. % zinc, and 0.01-1 wt. % zirconium.

29. The downhole well component as defined in claim 17, wherein said magnesium alloy includes over 50 wt. % magnesium and one or more metals selected from the group consisting of 0.1-3 wt. % zinc, 0.01-1 wt. % zirconium, 0.05-1 wt. % manganese, 0.0002-0.04 wt. % boron, and 0.4-0.7 wt. % bismuth.

30. The downhole well component as defined in claim 1, wherein said additive material includes nickel, said nickel constitutes 0.3-7 wt. % of said dissolvable magnesium cast material.

31. The downhole well component as defined in claim 1, wherein said additive material includes copper, said copper constitutes 0.5-15 wt. % of said dissolvable magnesium cast material.

32. The downhole well component as defined in claim 4, wherein said additive material includes copper, said copper constitutes 0.5-15 wt. % of said dissolvable magnesium cast material.

33. The downhole well component as defined in claim 9, wherein said additive material includes copper, said copper constitutes 0.5-15 wt. % of said dissolvable magnesium cast material.

34. The downhole well component as defined in claim 12, wherein said additive material includes copper, said copper constitutes 0.5-15 wt. % of said dissolvable magnesium cast material.

35. The downhole well component as defined in claim 11, wherein said additive material includes copper, said copper constitutes 0.5-15 wt. % of said dissolvable magnesium cast material.

36. The downhole well component as defined in claim 14, wherein said additive material includes copper, said copper constitutes 0.5-15 wt. % of said dissolvable magnesium cast material.

37. The downhole well component as defined in claim 1, wherein said downhole well component includes one or more components selected from the group consisting of a ball, tube, or plug.

38. The downhole well component as defined in claim 13, wherein said downhole well component includes one or more components selected from the group consisting of a sleeve, a ball, a frac ball, a hydraulic actuating tooling, a tube, a valve, a valve component, and a plug.

39. The downhole well component as defined in claim 14, wherein said downhole well component includes one or more components selected from the group consisting of a sleeve, a ball, a frac ball, a hydraulic actuating tooling, a tube, a valve, a valve component, and a plug.

40. The downhole well component as defined in claim 1, wherein said dissolvable magnesium cast material has one or more properties selected from the group consisting of a) a tensile strength of 14-50 ksi, b) a shear strength of 11-25 ksi, and c) an elongation of 3-12%.

41. The downhole well component as defined in claim 4, wherein said dissolvable magnesium cast material has one or more properties selected from the group consisting of a) a tensile strength of 14-50 ksi, b) a shear strength of 11-25 ksi, and c) an elongation of 3-12%.

42. The downhole well component as defined in claim 9, wherein said dissolvable magnesium cast material has one or more properties selected from the group consisting of a) a tensile strength of 14-50 ksi, b) a shear strength of 11-25 ksi, and c) an elongation of 3-12%.

43. The downhole well component as defined in claim 12, wherein said dissolvable magnesium cast material has one or more properties selected from the group consisting of a) a tensile strength of 14-50 ksi, b) a shear strength of 11-25 ksi, and c) an elongation of 3-12%.

44. The downhole well component as defined in claim 13, wherein said dissolvable magnesium cast material has one or more properties selected from the group consisting of a) a tensile strength of 14-50 ksi, b) a shear strength of 11-25 ksi, and c) an elongation of 3-12%.

45. The downhole well component as defined in claim 14, wherein said dissolvable magnesium cast material has one or more properties selected from the group consisting of a) a

tensile strength of 14-50 ksi, b) a shear strength of 11-25 ksi, and c) an elongation of 3-12%.

46. A downhole well component at least partially formed of a dissolvable magnesium cast material, said dissolvable magnesium cast material comprising a mixture of magnesium and additive material or a mixture of magnesium alloy and additive material, said dissolvable magnesium cast material includes at least 50 wt. % magnesium, said additive material added to said magnesium or magnesium alloy during formation of said dissolvable magnesium cast material, said additive material includes i) copper wherein said copper constitutes 0.5-15 wt. % of said dissolvable magnesium cast material and/or ii) nickel wherein said nickel constitutes 0.1-23.5 wt. % of said dissolvable magnesium cast material, said dissolvable magnesium cast material includes in situ precipitate, said in situ precipitate includes said additive material, said dissolvable magnesium cast material has a dissolution rate of at least 40 mg/cm<sup>2</sup>/hr. in 3 wt. % KCl water mixture at 90° C., said downhole well component including one or more components selected from the group consisting of a sleeve, a ball, a frac ball, a hydraulic actuating tooling, a tube, a valve, a valve component, and a plug.

47. The downhole well component as defined in claim 46, wherein said dissolvable magnesium cast material includes no more than 10 wt. % aluminum.

48. The downhole well component as defined in claim 46, wherein said dissolvable magnesium cast material has a dissolution rate of at least 75 mg/cm<sup>2</sup>/hr. in 3 wt. % KCl water mixture at 90° C.

49. The downhole well component as defined in claim 47, wherein said dissolvable magnesium cast material has a dissolution rate of at least 75 mg/cm<sup>2</sup>/hr. in 3 wt. % KCl water mixture at 90° C.

50. The downhole well component as defined in claim 46, wherein said dissolvable magnesium cast material includes at least 85 wt. % magnesium.

51. The downhole well component as defined in claim 48, wherein said dissolvable magnesium cast material includes at least 85 wt. % magnesium.

52. The downhole well component as defined in claim 49, wherein said dissolvable magnesium cast material includes at least 85 wt. % magnesium.

53. The downhole well component as defined in claim 49, wherein said magnesium alloy includes at least 85 wt. % magnesium and one or more metals selected from the group consisting of 0.5-10 wt. % aluminum, 0.05-6 wt. % zinc, 0.01-3 wt. % zirconium, and 0.15-2 wt. % manganese.

54. The downhole well component as defined in claim 52, wherein said magnesium alloy includes at least 85 wt. % magnesium and one or more metals selected from the group consisting of 0.5-10 wt. % aluminum, 0.05-6 wt. % zinc, 0.01-3 wt. % zirconium, and 0.15-2 wt. % manganese.

55. The downhole well component as defined in claim 46, wherein said magnesium alloy includes over 50 wt. % magnesium and one or more metals selected from the group consisting of aluminum, boron, bismuth, zinc, zirconium, and manganese.

56. The downhole well component as defined in claim 49, wherein said magnesium alloy includes over 50 wt. % magnesium and one or more metals selected from the group consisting of aluminum, boron, bismuth, zinc, zirconium, and manganese.

57. The downhole well component as defined in claim 55, wherein said magnesium alloy includes over 50 wt. % magnesium and one or more metals selected from the group consisting of aluminum in an amount of 0.5-10 wt. %, zinc

in an amount of 0.1-6 wt. %, zirconium in an amount of 0.01-3 wt. %, manganese in an amount of 0.15-2 wt. %, boron in an amount of 0.0002-0.04 wt. %, and bismuth in an amount of 0.4-0.7 wt. %.

58. The downhole well component as defined in claim 56, wherein said magnesium alloy includes over 50 wt. % magnesium and one or more metals selected from the group consisting of aluminum in an amount of 0.5-10 wt. %, zinc in an amount of 0.1-6 wt. %, zirconium in an amount of 0.01-3 wt. %, manganese in an amount of 0.15-2 wt. %, boron in an amount of 0.0002-0.04 wt. %, and bismuth in an amount of 0.4-0.7 wt. %.

59. The downhole well component as defined in claim 55, wherein said magnesium alloy comprises greater than 50 wt. % magnesium and one or more metals selected from the group consisting of 0.5-10 wt. % aluminum, 0.1-2 wt. % zinc, 0.01-1 wt. % zirconium, and 0.15-2 wt. % manganese.

60. The downhole well component as defined in claim 56, wherein said magnesium alloy comprises greater than 50 wt. % magnesium and one or more metals selected from the group consisting of 0.5-10 wt. % aluminum, 0.1-2 wt. % zinc, 0.01-1 wt. % zirconium, and 0.15-2 wt. % manganese.

61. The downhole well component as defined in claim 55, wherein said magnesium alloy comprises greater than 50 wt. % magnesium and one or more metals selected from the group consisting of 0.1-3 wt. % zinc, 0.05-1 wt. % zirconium, 0.05-0.25 wt. % manganese, 0.0002-0.04 wt. % boron, and 0.4-0.7 wt. % bismuth.

62. The downhole well component as defined in claim 56, wherein said magnesium alloy comprises greater than 50 wt. % magnesium and one or more metals selected from the group consisting of 0.1-3 wt. % zinc, 0.05-1 wt. % zirconium, 0.05-0.25 wt. % manganese, 0.0002-0.04 wt. % boron, and 0.4-0.7 wt. % bismuth.

63. The downhole well component as defined in claim 55, wherein said magnesium alloy comprises 60-95 wt. % magnesium, 0.5-10 wt. % aluminum, 0.05-6 wt. % zinc, and 0.15-2 wt. % manganese.

64. The downhole well component as defined in claim 56, wherein said magnesium alloy comprises 60-95 wt. % magnesium, 0.5-10 wt. % aluminum, 0.05-6 wt. % zinc, and 0.15-2 wt. % manganese.

65. The downhole well component as defined in claim 55, wherein said magnesium alloy includes 60-95 wt. % magnesium and 0.01-1 wt. % zirconium.

66. The downhole well component as defined in claim 56, wherein said magnesium alloy includes 60-95 wt. % magnesium and 0.01-1 wt. % zirconium.

67. The downhole well component as defined in claim 55, wherein said magnesium alloy includes 60-95 wt. % magnesium, 0.05-6 wt. % zinc, and 0.01-1 wt. % zirconium.

68. The downhole well component as defined in claim 56, wherein said magnesium alloy includes 60-95 wt. % magnesium, 0.05-6 wt. % zinc, and 0.01-1 wt. % zirconium.

69. The downhole well component as defined in claim 55, wherein said magnesium alloy includes over 50 wt. % magnesium and one or more metals selected from the group consisting of 0.1-3 wt. % zinc, 0.01-1 wt. % zirconium, 0.05-1 wt. % manganese, 0.0002-0.04 wt. % boron, and 0.4-0.7 wt. % bismuth.

70. The downhole well component as defined in claim 56, wherein said magnesium alloy includes over 50 wt. % magnesium and one or more metals selected from the group consisting of 0.1-3 wt. % zinc, 0.01-1 wt. % zirconium, 0.05-1 wt. % manganese, 0.0002-0.04 wt. % boron, and 0.4-0.7 wt. % bismuth.

71. The downhole well component as defined in claim 46, wherein said dissolvable magnesium cast material has a tensile strength of 14-50 ksi, a shear strength of 11-25 ksi, and an elongation of 3-12%.

5 72. The downhole well component as defined in claim 69, wherein said dissolvable magnesium cast material has a tensile strength of 14-50 ksi, a shear strength of 11-25 ksi, and an elongation of 3-12%.

10 73. The downhole well component as defined in claim 70, wherein said dissolvable magnesium cast material has a tensile strength of 14-50 ksi, a shear strength of 11-25 ksi, and an elongation of 3-12%.

15 74. A downhole well component at least partially formed of a dissolvable magnesium cast material, said dissolvable magnesium cast material comprising a mixture of magnesium and additive material or a mixture of magnesium alloy and additive material, said dissolvable magnesium cast material including includes at least 50 wt. % magnesium, said additive material is added to said magnesium or magnesium alloy during formation of said dissolvable magnesium cast material, said additive material includes nickel wherein said nickel constitutes 0.1-23.5 wt. % of said dissolvable magnesium cast material, said dissolvable magnesium cast material includes in situ precipitate, said in situ precipitate includes said additive material, said dissolvable magnesium cast material has a dissolution rate of at least 40 mg/cm<sup>2</sup>/hr. in 3 wt. % KCl water mixture at 90° C.

20 75. The downhole well component as defined in claim 74, wherein said dissolvable magnesium cast material includes no more than 10 wt. % aluminum.

25 76. The downhole well component as defined in claim 74, wherein said dissolvable magnesium cast material has a dissolution rate of at least 75 mg/cm<sup>2</sup>/hr. in 3 wt. % KCl water mixture at 90° C.

30 77. The downhole well component as defined in claim 75, wherein said dissolvable magnesium cast material has a dissolution rate of at least 75 mg/cm<sup>2</sup>/hr. in 3 wt. % KCl water mixture at 90° C.

78. The downhole well component as defined in claim 74, wherein said dissolvable magnesium cast material includes at least 85 wt. % magnesium.

45 79. The downhole well component as defined in claim 75, wherein said dissolvable magnesium cast material includes at least 85 wt. % magnesium.

80. The downhole well component as defined in claim 76, wherein said dissolvable magnesium cast material includes at least 85 wt. % magnesium.

50 81. The downhole well component as defined in claim 77, wherein said dissolvable magnesium alloy includes at least 85 wt. % magnesium.

82. The downhole well component as defined in claim 74, wherein said downhole well component including includes 55 one or more components selected from the group consisting of a sleeve, a ball, a frac ball, a hydraulic actuating tooling, a tube, a valve, a valve component, and a plug.

60 83. The downhole well component as defined in claim 77, wherein said downhole well component including includes one or more components selected from the group consisting of a sleeve, a ball, a frac ball, a hydraulic actuating tooling, a tube, a valve, a valve component, and a plug.

65 84. The downhole well component as defined in claim 81, wherein said downhole well component including includes one or more components selected from the group consisting of a sleeve, a ball, a frac ball, a hydraulic actuating tooling, a tube, a valve, a valve component, and a plug.

## 25

**85.** The downhole well component as defined in claim **74**, wherein said dissolvable magnesium cast material has a tensile strength of 14-50 ksi, a shear strength of 11-25 ksi, and an elongation of 3-12%.

**86.** The downhole well component as defined in claim **82**, wherein said dissolvable magnesium cast material has a tensile strength of 14-50 ksi, a shear strength of 11-25 ksi, and an elongation of 3-12%.

**87.** The downhole well component as defined in claim **83**, wherein said dissolvable magnesium cast material has a tensile strength of 14-50 ksi, a shear strength of 11-25 ksi, and an elongation of 3-12%.

**88.** The downhole well component as defined in claim **83**, wherein said dissolvable magnesium cast material has a tensile strength of 14-50 ksi, a shear strength of 11-25 ksi, and an elongation of 3-12%.

**89.** A downhole well component at least partially formed of a dissolvable magnesium cast material, said dissolvable magnesium cast material comprising a mixture of magnesium alloy and additive material, said magnesium alloy includes at least 85 wt. % magnesium and one or more metals selected from the group consisting of aluminum, boron, bismuth, zinc, zirconium, and manganese, said additive material added to said magnesium alloy during formation of said dissolvable magnesium cast material, said additive material includes nickel wherein said nickel constitutes at least 0.01 wt. % of said dissolvable magnesium cast material, said dissolvable magnesium cast material includes in situ precipitate, said in situ precipitate includes said additive material, said dissolvable magnesium cast material has a dissolution rate of at least 75 mg/cm<sup>2</sup>/hr. in 3 wt. % KCl water mixture at 90° C., said downhole well component includes one or more components selected from the group

## 26

consisting of a sleeve, a ball, a frac ball, a hydraulic actuating tooling, a tube, a valve, a valve component, and a plug.

**90.** The downhole well component as defined in claim **89**, wherein said dissolvable magnesium cast material includes no more than 10 wt. % aluminum.

**91.** The downhole well component as defined in claim **89**, wherein said nickel constitutes 0.01-5 wt. % of said dissolvable magnesium cast material.

**92.** The downhole well component as defined in claim **90**, wherein said nickel constitutes 0.01-5 wt. % of said dissolvable magnesium cast material.

**93.** The downhole well component as defined in claim **89**, wherein said nickel constitutes 0.1-24.5 wt. % of said dissolvable magnesium cast material.

**94.** The downhole well component as defined in claim **90**, wherein said nickel constitutes 0.1-24.5 wt. % of said dissolvable magnesium cast material.

**95.** The downhole well component as defined in claim **89**, wherein said in situ precipitate has a size of less than 50 µm.

**96.** The downhole well component as defined in claim **90**, wherein said in situ precipitate has a size of less than 50 µm.

**97.** The downhole well component as defined in claim **91**, wherein said in situ precipitate has a size of less than 50 µm.

**98.** The downhole well component as defined in claim **92**, wherein said in situ precipitate has a size of less than 50 µm.

**99.** The downhole well component as defined in claim **93**, wherein said in situ precipitate has a size of less than 50 µm.

**100.** The downhole well component as defined in claim **94**, wherein said in situ precipitate has a size of less than 50 µm.

\* \* \* \* \*